



US011053602B2

(12) **United States Patent**  
Sung et al.

(10) **Patent No.:** US 11,053,602 B2  
(45) **Date of Patent:** \*Jul. 6, 2021

(54) **MICRO-ROUGHENED  
ELECTRODEPOSITED COPPER FOIL AND  
COPPER FOIL SUBSTRATE**

(71) Applicant: **CO-TECH DEVELOPMENT CORP.**,  
Taipei (TW)

(72) Inventors: **Yun-Hsing Sung**, Taoyuan (TW);  
**Chun-Yu Kao**, Yunlin County (TW)

(73) Assignee: **CO-TECH DEVELOPMENT CORP.**,  
Taipei (TW)

(\*) Notice: Subject to any disclaimer, the term of this  
patent is extended or adjusted under 35  
U.S.C. 154(b) by 60 days.

This patent is subject to a terminal dis-  
claimer.

(21) Appl. No.: **16/563,954**

(22) Filed: **Sep. 9, 2019**

(65) **Prior Publication Data**

US 2020/0087811 A1 Mar. 19, 2020

(30) **Foreign Application Priority Data**

Sep. 17, 2018 (TW) ..... 107132627

(51) **Int. Cl.**

**B21C 37/00** (2006.01)  
**C25D 7/06** (2006.01)

(Continued)

(52) **U.S. Cl.**

CPC ..... **C25D 7/0614** (2013.01); **C25D 1/04**  
(2013.01); **C25D 3/38** (2013.01); **C25D 5/16**  
(2013.01); **Y10T 428/12431** (2015.01)

(58) **Field of Classification Search**

None

See application file for complete search history.

(56) **References Cited**

U.S. PATENT DOCUMENTS

6,291,081 B1 \* 9/2001 Kurabe ..... C25D 1/04  
2004/0108211 A1 6/2004 Chiu et al. 174/257  
(Continued)

FOREIGN PATENT DOCUMENTS

CN 1543292 A 11/2004  
CN 101935856 A 1/2011  
(Continued)

OTHER PUBLICATIONS

Merriam-Webster, "Definition of length", <https://www.merriam-webster.com/dictionary/length>, accessed May 6, 2020 (Year: 2020)  
(Year: 2020).\*

(Continued)

*Primary Examiner* — Seth Dumbris

(74) *Attorney, Agent, or Firm* — Li & Cai Intellectual  
Property Office

(57) **ABSTRACT**

A micro-roughened electrodeposited copper foil and a copper foil substrate are provided. The micro-roughened electrodeposited copper foil includes a micro-rough surface. The micro-rough surface has a plurality of peaks, a plurality of V-shaped grooves and a plurality of micro-crystal clusters. Each of the V-shaped grooves is defined by adjacent two of the peaks and has an average depth less than 1  $\mu\text{m}$ . The micro-crystal clusters are correspondingly located on the tops of the peaks and each thereof has an average height less than 1.5  $\mu\text{m}$ . The micro-rough surface of the micro-roughened electrodeposited copper foil has an Rlr value less than 1.06.

**12 Claims, 9 Drawing Sheets**



---

|      |                  |           |  |    |             |         |
|------|------------------|-----------|--|----|-------------|---------|
| (51) | <b>Int. Cl.</b>  |           |  |    |             |         |
|      | <i>C25D 3/38</i> | (2006.01) |  | CN | 102534710 A | 7/2012  |
|      | <i>C25D 5/16</i> | (2006.01) |  | CN | 102618902 A | 8/2012  |
|      | <i>C25D 1/04</i> | (2006.01) |  | CN | 106011965 A | 10/2016 |

**(56) References Cited**

## U.S. PATENT DOCUMENTS

|                  |        |               |           |
|------------------|--------|---------------|-----------|
| 2005/0175826 A1* | 8/2005 | Suzuki .....  | C25D 1/04 |
|                  |        |               | 428/209   |
| 2009/0047539 A1* | 2/2009 | Dobashi ..... | C25D 1/04 |
|                  |        |               | 428/607   |
| 2012/0189859 A1* | 7/2012 | Nozaki .....  | H05K 1/09 |
|                  |        |               | 428/458   |

## FOREIGN PATENT DOCUMENTS

|    |             |        |
|----|-------------|--------|
| CN | 102418129 A | 4/2012 |
| CN | 102482795 A | 5/2012 |

## OTHER PUBLICATIONS

K. C. Yung, J. Wang and T. M. Yue, "Surface characterization of pre-treated copper foil used for PCB lamination", *J. Adhesion Sol. Technol.*, vol. 21, No. 5-6, Apr. 2, 2012 (Apr. 2, 2012), pp. 363-377.

\* cited by examiner



FIG. 1



FIG. 2



FIG. 3



FIG. 4



FIG. 5



FIG. 6



FIG. 7



FIG. 8



FIG. 9

## 1

**MICRO-ROUGHENED  
ELECTRODEPOSITED COPPER FOIL AND  
COPPER FOIL SUBSTRATE**

**CROSS-REFERENCE TO RELATED PATENT  
APPLICATION**

This application claims the benefit of priority to Taiwan Patent Application No. 107132627, filed on Sep. 17, 2018. The entire content of the above identified application is incorporated herein by reference.

Some references, which may include patents, patent applications and various publications, may be cited and discussed in the description of this disclosure. The citation and/or discussion of such references is provided merely to clarify the description of the present disclosure and is not an admission that any such reference is "prior art" to the disclosure described herein. All references cited and discussed in this specification are incorporated herein by reference in their entireties and to the same extent as if each reference was individually incorporated by reference.

**FIELD OF THE DISCLOSURE**

The present disclosure relates to a copper foil, and more particularly to an electrodeposited copper foil and a copper foil substrate having the electrodeposited copper foil.

**BACKGROUND OF THE DISCLOSURE**

With the development of information and electronic industries, high-frequency and high-speed signal transmission has become an integral part of modern circuit design and manufacture. In order to meet the high-frequency and high-speed signal transmission requirements of electronic products, the copper foil substrate used needs to have a good insertion loss performance at high frequencies so as to transmit high-frequency signals without excessive loss. The insertion loss of the copper foil substrate is highly correlated with its surface roughness. The copper foil substrate has a good insertion loss performance when the surface roughness is decreased, or otherwise does not. However, the decrease of the surface roughness may reduce the peel strength between the copper foil and the substrate. Therefore, how the peel strength can be maintained at the industry level and provide good insertion loss performance has become a problem to be solved in the related field.

**SUMMARY OF THE DISCLOSURE**

In response to the above-referenced technical inadequacies, the present disclosure provides a micro-roughened electrodeposited copper foil.

In one aspect, the present disclosure provides a micro-roughened electrodeposited copper foil. The micro-roughened electrodeposited copper foil includes a micro-rough surface. The micro-rough surface has a plurality of peaks, a plurality of V-shaped grooves and a plurality of micro-crystal clusters. Each of the V-shaped grooves has an average depth less than 1  $\mu\text{m}$  and is defined by an adjacent two of the peaks. The micro-crystal clusters are correspondingly located on the tops of the peaks and each thereof has an average height less than 1.5  $\mu\text{m}$ . The micro-rough surface of the micro-roughened electrodeposited copper foil has an Rlr value less than 1.06.

In certain embodiments, each of the micro-crystal clusters is composed of a plurality of micro-crystals grouped

## 2

together and has an average height less than 1.3  $\mu\text{m}$ . Each of the micro-crystals has an average diameter less than 0.5  $\mu\text{m}$ .

In certain embodiments, each of the micro-crystal clusters has an average number of the micro-crystals, which are stacked in a height direction thereof, less than 15. Each of the micro-crystal clusters has an average maximum width less than 5  $\mu\text{m}$ , and a portion of the micro-crystal clusters are formed with a branch structure.

In certain embodiments, the Rlr value the micro-rough surface of the micro-roughened electrodeposited copper foil is less than 1.055.

In one aspect, the present disclosure provides a copper foil substrate which includes a substrate and a micro-roughened electrodeposited copper foil. The micro-roughened electrodeposited copper foil includes a micro-rough surface attached to the substrate. The micro-rough surface has a plurality of peaks, a plurality of V-shaped grooves and a plurality of micro-crystal clusters. Each of the V-shaped grooves has an average depth less than 1  $\mu\text{m}$  and is defined by adjacent two of the peaks. The micro-crystal clusters are correspondingly located on the tops of the peaks and each thereof has an average height less than 1.5  $\mu\text{m}$ . The copper foil substrate has an insertion loss between 0 and -0.635 dB/in at 20 GHz. The micro-roughened electrodeposited copper foil has a peel strength greater than 3 lb/in relative to the substrate.

In certain embodiments, the copper foil substrate has an insertion loss between 0 and -0.935 dB/in at 30 GHz.

In certain embodiments, the copper foil substrate has an insertion loss between 0 and -0.31 dB/in at 8 GHz. The copper foil substrate has an insertion loss between 0 and -0.43 dB/in at 12.89 GHz. The copper foil substrate has an insertion loss between 0 and -0.53 dB/in at 16 GHz. The peel strength of the micro-roughened electrodeposited copper foil relative to the substrate is greater than 3.5 lb/in.

In certain embodiments, the insertion loss of the copper foil substrate at 12.89 GHz is between 0 and -0.42 dB/in. The insertion loss of the copper foil substrate at 16 GHz is between 0 and -0.52 dB/in. The insertion loss of the copper foil substrate at 20 GHz is between 0 and -0.63 dB/in. The insertion loss of the copper foil substrate at 30 GHz is between 0 and -0.92 dB/in. The peel strength of the copper foil substrate relative to the substrate is greater than 3.9 lb/in.

In certain embodiments, each of the micro-crystal clusters has an average maximum width less than 5  $\mu\text{m}$ . A portion of the micro-crystal clusters are formed with a branch structure. The average height of each of the micro-crystal clusters is less than 1  $\mu\text{m}$ . Each of the micro-crystal clusters is composed of a plurality of micro-crystals grouped together. Each of the micro-crystals has an average diameter less than 0.5  $\mu\text{m}$ . The micro-rough surface of the micro-roughened electrodeposited copper foil has an Rlr value less than 1.06.

In certain embodiments, the substrate has a dielectric constant (Dk) less than 3.8 and a dissipation factor (Df) less than 0.002 at 1 GHz.

One of the advantages of the present disclosure is that the micro-rough surface has good bonding strength relative to the substrate, and the copper foil substrate has good performance on insertion loss at high frequencies and can effectively reduce the transmission loss of signals.

These and other aspects of the present disclosure will become apparent from the following description of the embodiment taken in conjunction with the following drawings and their captions, although variations and modifica-

tions therein may be affected without departing from the spirit and scope of the novel concepts of the disclosure.

#### BRIEF DESCRIPTION OF THE DRAWINGS

The present disclosure will become more fully understood from the following detailed description and accompanying drawings.

FIG. 1 is a side schematic view showing an implementation example of a copper foil substrate of the present disclosure.

FIG. 2 is an enlarged view of part II of FIG. 1.

FIG. 3 is a schematic view showing a production apparatus of a micro-roughened electrolysis copper foil.

FIG. 4 is a scanning electron microscope image showing a surface profile of the micro-roughened electrolysis copper foil of Example 1.

FIG. 5 is a scanning electron microscope image showing a cross-section profile of the micro-roughened electrolysis copper foil of Example 1.

FIG. 6 is a scanning electron microscope image showing a surface profile of a copper foil of Comparative Example 3.

FIG. 7 is a scanning electron microscope image showing a cross-section profile of the copper foil of Comparative Example 3.

FIG. 8 is a scanning electron microscope image showing a surface profile of a copper foil of Comparative Example 4.

FIG. 9 is a scanning electron microscope image showing a cross-section profile of the copper foil of Comparative Example 4.

#### DETAILED DESCRIPTION OF THE EXEMPLARY EMBODIMENTS

The present disclosure is more particularly described in the following examples that are intended as illustrative only since numerous modifications and variations therein will be apparent to those skilled in the art. Like numbers in the drawings indicate like components throughout the views. As used in the description herein and throughout the claims that follow, unless the context clearly dictates otherwise, the meaning of "a", "an", and "the" includes plural reference, and the meaning of "in" includes "in" and "on". Titles or subtitles can be used herein for the convenience of a reader, which shall have no influence on the scope of the present disclosure.

The terms used herein generally have their ordinary meanings in the art. In the case of conflict, the present document, including any definitions given herein, will prevail. The same thing can be expressed in more than one way. Alternative language and synonyms can be used for any term(s) discussed herein, and no special significance is to be placed upon whether a term is elaborated or discussed herein. A recital of one or more synonyms does not exclude the use of other synonyms. The use of examples anywhere in this specification including examples of any terms is illustrative only, and in no way limits the scope and meaning of the present disclosure or of any exemplified term. Likewise, the present disclosure is not limited to various embodiments given herein. Numbering terms such as "first", "second" or "third" can be used to describe various components, signals or the like, which are for distinguishing one component/signal from another one only, and are not intended to, nor should be construed to impose any substantive limitations on the components, signals or the like.

Referring to FIG. 1, a copper foil substrate 1 of the present disclosure includes a substrate 11 and two micro-roughened electrodeposited copper foils 12. The micro-roughened electrodeposited copper foils 12 are respectively attached to two opposite sides of the substrate. It is worth mentioning that,

the copper foil substrate 1 can include only one micro-roughened electrodeposited copper foil 12.

The substrate 11 has a low dielectric constant (Dk) and a low dissipation factor (Df) so as to reduce insertion loss. Preferably, the substrate 11 has a Dk less than 4 and a Df less than 0.003. More preferably, the substrate 11 has a Dk less than 3.8 and a Df less than 0.002.

The substrate 11 can be made from a composite material which is prepared by impregnating a base material with a synthetic resin. The base material may be, for example, a phenolic cotton paper, cotton paper, resin fiber fabric, resin fiber non-woven fabric, glass board, glass woven fabric, or glass non-woven fabric. The synthetic resin may, for example, be an epoxy resin, polyester resin, polyimide resin, cyanate ester resin, bismaleimide triazine resin, polyphenylene ether resin, or phenol resin. The synthetic resin layer may be formed into a single layer or multi layers, but is not limited thereto. The substrate 11 may be made from, but not limited to, EM891, IT958G, IT150DA, S7439G, MEGTRON 4, MEGTRON 6, or MEGTRON 7.

Referring to FIG. 1 along with FIG. 2, the micro-roughened electrodeposited copper foil 12 is obtained by using an electrolysis method to roughen a surface of a copper foil. The electrolysis method can be used to roughen any one surface of the copper foil, such that the micro-roughened electrodeposited copper foil 12 has a micro-rough surface 121 on at least one side thereof. In one embodiment of the present disclosure, a very low profile (VLP) copper foil is used as a raw foil and subsequently a rough surface thereof is roughened to obtain the micro-roughened electrodeposited copper foil 12.

The micro-rough surface 121 is configured to attach to the substrate 11, and includes a plurality of peaks 122, a plurality of V-shaped grooves 123 and a plurality of micro-crystal clusters 124. Each of the V-shaped grooves 123 is defined by adjacent two of the peaks 122. The V-shaped groove 123 has an average depth less than 1.5  $\mu\text{m}$ , preferably less than 1.3  $\mu\text{m}$ , and more preferably less than 1  $\mu\text{m}$ . The V-shaped groove 123 has an average width less than 1.5  $\mu\text{m}$ , preferably less than 1.3  $\mu\text{m}$ , and more preferably less than 1  $\mu\text{m}$ .

The micro-crystal cluster 124 has an average height less than 1.5  $\mu\text{m}$ , preferably less than 1.3  $\mu\text{m}$ , and more preferably less than 1  $\mu\text{m}$ . The aforesaid "average height" refers to a distance from the top of the micro-crystal cluster 124 to the top of the corresponding peak 122. The micro-crystal cluster 124 has an average maximum width less than 5  $\mu\text{m}$ , preferably less than 3  $\mu\text{m}$ . Each of the micro-crystal clusters 124 is composed of a plurality of micro-crystals 125 grouped together. Each of the micro-crystals 125 has an average diameter less than or equal to 0.5  $\mu\text{m}$ , preferably between 0.05  $\mu\text{m}$  to 0.5  $\mu\text{m}$ , and more preferably between 0.1  $\mu\text{m}$  to 0.4  $\mu\text{m}$ . Each of the micro-crystal clusters 124 has an average number of the micro-crystals 125 stacked in a height direction thereof less than 15, preferably less than 13, more preferably less than 10, and most preferably less than 8. When the micro-crystals 125 are grouped together to form the micro-crystal cluster 124, they can be stacked into a tower structure or a branch structure extending outwardly.

There is no limitation on the arrangement among the micro-crystal clusters 124. The micro-crystal clusters 124 can be arranged in an irregular manner or be substantially arranged along the same direction. In addition, a number of the micro-crystal clusters 124 can be arranged into a row and a portion of the rows have the same extension direction.

The micro-rough surface 121 of the micro-roughened electrodeposited copper foil 12 has an average roughness Rz greater than 0.5  $\mu\text{m}$ , preferably greater than 1.0  $\mu\text{m}$ , and more preferably greater than 1.2  $\mu\text{m}$ . When the average roughness Rz of the micro-rough surface 121 satisfies the above ranges, the micro-roughened electrodeposited copper foil 12 has good bonding strength relative to the substrate 11.

That is to say, the increase of the average roughness  $R_z$  can improve the bonding strength between the micro-roughened electrodeposited copper foil **12** and the substrate **11**, and thus significantly increase the peel strength. The peel strength between the micro-roughened electrodeposited copper foil **12** and the substrate **11** can be greater than 3 lb/in, preferably greater than 3.2 lb/in, more preferably greater than 3.5 lb/in, and most preferably greater than 3.7 lb/in. It is worth mentioning that, when an adhesive is applied to the micro-rough surface **11**, the adhesive would permeate into the V-shaped grooves **123** and the bottoms of the micro-crystal clusters **124**, such that the peel strength of the micro-roughened electrodeposited copper foil **12** after adhering to the substrate **11** can be significantly increased.

By the profile of the micro-rough surface **121**, the micro-roughened electrodeposited copper foil **12** can have enough peel strength relative to the substrate **11** and can significantly reduce the signal transmission loss. The micro-rough surface **121** has an  $R_{lr}$  value less than 1.06, preferably less than 1.055, and more preferably less than 1.05. The term “ $R_{lr}$  value” refers to an expanded length ratio, i.e., a length ratio of the surface profile of the test object per unit length. A higher  $R_{lr}$  value indicates that the surface profile is more uneven, and the surface is completely flat when the value is equal to 1. The  $R_{lr}$  value satisfies the equation of  $R_{lr}=R_{lo}/L$ ;  $R_{lo}$  represents a measured profile length;  $L$  represents a measured distance. The  $R_{lr}$  value of the micro-roughened electrodeposited copper foil **12** is measured by a shape measurement laser microscope (“VK-X100” made by Keyence Corporation), and the cut-off wavelengths  $\lambda_s$  and  $\lambda_c$  for measurement are respectively 2.5  $\mu\text{m}$  and 0.003 mm.

When the micro-roughened electrodeposited copper foil **12** has the above  $R_{lr}$  values, the copper foil substrate **1** would have good insertion loss performance. The copper foil substrate **1** has an insertion loss between 0 and  $-0.31$  dB/in at 8 GHz, preferably between 0 and  $-0.305$  dB/in. The copper foil substrate **1** has an insertion loss between 0 and  $-0.43$  dB/in at 12.89 GHz, preferably between 0 and  $-0.42$  dB/in, and more preferably between 0 and  $-0.41$  dB/in. The copper foil substrate **1** has an insertion loss between 0 and  $-0.53$  dB/in at 16 GHz, preferably between 0 and  $-0.52$  dB/in, and more preferably between 0 and  $-0.51$  dB/in. The copper foil substrate **1** has an insertion loss between 0 and  $-0.635$  dB/in at 20 GHz, preferably between 0 and  $-0.63$  dB/in, more preferably between 0 and  $-0.62$  dB/in, still more preferably between 0 and  $-0.61$  dB/in, and most preferably between 0 and  $-0.6$  dB/in. The copper foil substrate **1** has an insertion loss between 0 and  $-0.78$  dB/in at 25 GHz, preferably between 0 and  $-0.77$  dB/in, more preferably between 0 and  $-0.76$  dB/in, and most preferably between 0 and  $-0.74$  dB/in. The copper foil substrate **1** has an insertion loss between 0 and  $-0.935$  dB/in at 30 GHz, preferably between 0 and  $-0.92$  dB/in, more preferably between 0 and  $-0.90$  dB/in, and most preferably between 0 and  $-0.88$  dB/in. In this description, the insertion loss is represented by a negative value. The micro-roughened electrodeposited copper foil **12** of the present disclosure can effectively reduce the signal transmission loss at high frequencies, particularly at 16 GHz or more.

#### [Manufacturing Method of Micro-Roughened Electrodeposited Copper Foil]

The micro-roughened electrodeposited copper foil **12** is obtained by immersing a raw foil in a copper-containing plating solution and subsequently conducting an electrolytic roughening treatment in a predetermined period of time. In certain embodiments of the present disclosure, a very low profile (VLP) copper foil is used as a raw foil and subsequently a rough surface thereof is roughened. The electrolytic roughening treatment can be performed by any conventional apparatus such as a continuous-type or batch-type electrolyzing apparatus.

The copper-containing plating solution contains copper ions, an acid component and a metal additive. The source of copper ions may be exemplified by copper sulfate, copper nitrate, or the combination thereof. The acid component may be exemplified by sulfuric acid, nitric acid, or the combination thereof. The metal additive may be exemplified by cobalt, iron, zinc, or the combination thereof. In addition, the copper-containing plating solution can further contain any conventional additive such as gelatin, organic nitride, hydroxyethyl cellulose (HEC), polyethylene glycol (PEG), sodium 3-mercaptopropane sulphonate (MPS), Bis-(sodium sulfopropyl)-disulfide (SPS), or thiourea-containing compounds, but is not limited thereto.

The electrolytic roughening treatment can be performed twice with the same or different copper-containing plating solutions. In one embodiment of the present disclosure, two different copper-containing plating solutions (i.e., first and second copper-containing plating solutions) are alternately used for the electrolytic roughening treatments. The first copper-containing plating solution has a copper ion concentration between 10 g/L and 30 g/L, an acid concentration between 70 g/L and 100 g/L, and a metal additive concentration between 150 mg/L and 300 mg/L. The metal additive concentration is preferably between 15 mg/L and 100 mg/L. The second copper-containing plating solution has a copper ion concentration between 70 g/L and 100 g/L, an acid concentration between 30 g/L and 60 g/L, and a metal additive concentration between 15 mg/L and 100 mg/L.

The power required for the electrolytic roughening treatment can be supplied via a constant voltage, constant current, pulse wave, or saw wave manner, but is not limited thereto. In one embodiment of the present disclosure, for the electrolytic roughening treatments, the first copper-containing plating solution is used at a constant current density between 18 A/dm<sup>2</sup> and 40 A/dm<sup>2</sup> and subsequently the second copper-containing plating solution is used at a constant current density between 2.2 A/dm<sup>2</sup> and 5 A/dm<sup>2</sup>. Preferably, the first copper-containing plating solution is used at a constant current density between 20 A/dm<sup>2</sup> and 33 A/dm<sup>2</sup> and the second copper-containing plating solution is used at a constant current density between 2.7 A/dm<sup>2</sup> and 3 A/dm<sup>2</sup>. It is worth mentioning that, said constant current densities can be applied with a pulse or saw wave. In addition, if the power for the electrolytic roughening treatment is supplied with different constant voltages, each of the constant voltages must cause the current density to fall within the above current density ranges in the corresponding electrolytic roughening treatment.

When the electrolytic roughening treatment is performed thrice or more, the first and second copper-containing plating solutions can be alternately used for the electrolytic roughening treatments at a current density between 10 A/dm<sup>2</sup> and 16 A/dm<sup>2</sup>. In one embodiment of the present disclosure, the first copper-containing plating solution and the second copper-containing plating solution are respectively used for the third and fourth electrolytic roughening treatments at a current density between 13 A/dm<sup>2</sup> and 15 A/dm<sup>2</sup>. The fifth and later electrolytic roughening treatments are performed at a current density less than 5 A/dm<sup>2</sup>, preferably at different current densities that are decreased in order. It is worth mentioning that, said constant current densities can be applied with a pulse or saw wave. In addition, if the power for the electrolytic roughening treatment is supplied with different constant voltages, each of the constant voltages must cause the current density to fall within the above current density ranges in the corresponding electrolytic roughening treatment.

It is worth mentioning that, the arrangement of the micro-crystal clusters **124** of the micro-rough surface **121** and the extension direction of the V-shaped grooves **123** can be controlled by a flow field of the copper-containing plating solution(s). When no flow field or a turbulent flow is

generated, the micro-crystal clusters 124 are arranged in an irregular manner. When the flow field is generated along a predetermined direction, the micro-crystal clusters are substantially arranged along the same direction. However, the control manner of the arrangement of the micro-crystal clusters 124 and the extension direction of the V-shaped grooves 123 are limited to such details. In addition, it is also possible to use a steel brush to pre-scratch the non-oriented V-shaped grooves 123 or be adjusted to use any other conventional techniques as deemed fit by the manufacturer.

In one embodiment of the present disclosure, a continuous-type electrolyzing apparatus, which includes a plurality of tanks and a plurality of electrolyzing rolls, can be used to perform the electrolytic roughening treatment(s). The first copper-containing plating solution and the second copper-containing plating solution are alternately accommodated in the tanks. The electrolysis power is supplied with constant voltage(s). The production speed is controlled at 5-20 m/min and the production temperature is controlled at 20-60° C.

It should be noted that, the above method for manufacturing the micro-roughened electrodeposited copper foil can be applied to the high-temperature-elongation (HTE) copper foil and the reverse treated copper foil (RTF). The micro-roughened electrodeposited copper foil can be obtained by performing an electrolytic roughening treatment on a shiny side of a HTE copper foil.

The structure and the manufacturing method of each layer of the copper foil substrate 1 are described above. The following will provide Examples 1-3 and comparisons among Examples 1-3 and Comparative Examples 1-4, and further describe the advantages of the present disclosure.

#### Example 1

Referring to FIG. 3, a continuous-type electrolyzing apparatus 2 is shown. The continuous-type electrolyzing apparatus 2 can be used to perform electrolytic roughening treatment(s) so as to form a micro-roughened electrodeposited copper foil. The continuous-type electrolyzing apparatus 2 includes a feeding roll 21, a receiving roll 22, six tanks 23 (i.e., first to sixth tanks) arranged between the feeding roll 21 and the receiving roll 22, six electrolyzing roll assemblies 24 respectively arranged above the tanks 23, and six auxiliary roll assemblies 25 respectively arranged in the tanks 23. Each of the tanks 23 has a pair of platinum electrodes 231 arranged therein. Each of the electrolyzing roll assemblies 24 includes two electrolyzing rolls 241. Each of the auxiliary roll assemblies 25 includes two auxiliary rolls 251. The pair of platinum electrodes 231 in each of the tanks 23 and the corresponding electrolyzing roll assembly 24 are electrically connected to an anode and a cathode of an outer power supply, respectively.

In this example, a VLP copper foil (product name "VL410", purchased from Co-Tech Copper Foil Company) is used as a raw foil. The raw foil is rolled up on the feeding roll 21 and pulled tightly around the electrolyzing roll assemblies 24 and the auxiliary roll assemblies 25 in order, and is subsequently rolled up on the receiving roll 22. The copper-containing plating solution in each of the tanks is shown in Table 1, wherein the source of copper ions is copper sulfate. The raw foil sequentially passes through the first to sixth tanks 23 at a production speed of 10 m/min to roughen a matte side thereof. Accordingly, micro-roughened electrolysis copper foils each having a surface roughness  $R_z$ (JIS B0601-1994) of 1.29 are obtained. Finally, two of the micro-roughened electrolysis copper foils are attached to a Megtron 7 substrate, so as to form a copper foil substrate.

The surface and the cross-sectional structures of the micro-roughened electrolysis copper foil of Example 1 observed by a scanning electron microscope are shown in FIG. 4 and FIG. 5 respectively.

The micro-roughened electrolysis copper foil of Example 1, in which the micro-rough surface is coated with a silane coupling agent, is adhered to the Megtron 7 substrate. After curing, the IPC-TM-650 2.4.8 test method is used for peel strength measurement. The result is shown in Table 2.

The  $R_{lr}$  value of the micro-roughened electrolysis copper foil of Example 1 is measured by a shape measurement laser microscope ("VK-X100" made by Keyence Corporation). The result is shown in Table 2.

The insertion loss of the micro-roughened electrolysis copper foil of Example 1 is measured by a microstrip line having a characteristic impedance 50 ohms at 4 GHz, 8 GHz, 12.89 GHz, 16 GHz, 20 GHz, 25 GHz and 30 GHz. The results are shown in Table 2.

#### Examples 2 and 3

The raw foil, the electrolyzing apparatus and the composition of the copper-containing plating solution are the same as in Example 1. The electroplating conditions are shown in Table 1 and the production speed is 10 m/min. Two of the micro-roughened electrolysis copper foils of Example 2 and 3 are attached to a Megtron 7 substrate. The copper foil substrates obtained are measured in the same ways as in Example 1, and the results are shown in Table 2.

#### Comparative Examples 1 and 2

The raw foil, the electrolyzing apparatus and the composition of the copper-containing plating solution are the same as in Example 1. The electroplating conditions are shown in Table 1 and the production speed is 10 m/min. Two of the micro-roughened electrolysis copper foils of Comparative Examples 1 and 2 are attached to a Megtron 7 substrate. The copper foil substrates obtained are measured in the same ways as in Example 1, and the results are shown in Table 2.

#### Comparative Example 3

Comparative Example 3 uses very low profile (VLP) copper foils (trade name "CF-T4X-SV", from Fukuda Metal Foil Powder Co. Ltd., hereinafter "CF-T4X-SV copper foil"). The surface and the cross-sectional structures of the CF-T4X-SV copper foil are observed by a scanning electron microscope, which are shown in FIG. 6 and FIG. 7 respectively. Two of the CF-T4X-SV copper foils are attached to a Megtron 7 substrate so as to obtain a copper foil substrate, the peel strength,  $R_{lr}$  value and insertion loss of which are measured in the same ways as in Example 1, and the results are shown in Table 2.

#### Comparative Example 4

Comparative Example 4 uses very low profile (VLP) copper foils (product name "HS1-M2-VSP", from Taiwan Copper Foil Co., Ltd, hereinafter "HS1-M2-VSP copper foil"). The surface and the cross-sectional structures of the HS1-M2-VSP copper foil are observed by a scanning electron microscope, which are shown in FIG. 8 and FIG. 9 respectively. Two of the HS1-M2-VSP copper foils are attached to a Megtron 7 substrate to obtain a copper foil substrate, the peel strength,  $R_{lr}$  value and insertion loss of which are measured in the same ways as in Example 1, and the results are shown in Table 2.

TABLE 1

|                                      | First tank | Second tank | Third tank | Fourth tank | Fifth tank | Sixth tank |
|--------------------------------------|------------|-------------|------------|-------------|------------|------------|
| Cu <sup>+2</sup> (g/L)               | 15.5~20.5  | 86.5~90.5   | 15.5~20.5  | 86.5~90.5   | 15.5~20.5  | 86.5~90.5  |
| Cl (ppm)                             | <3         | <3          | <3         | <3          | <3         | <3         |
| H <sub>2</sub> SO <sub>4</sub> (g/L) | 83~87      | 45~55       | 83~87      | 45~55       | 83~87      | 45~55      |
| Metal additive (ppm)                 | 180~220    | 30~40       | 180~220    | 30~40       | 180~220    | 30~40      |
| Example 1 (A/dm <sup>2</sup> )       | 27.78      | 2.47        | 13.89      | 13.89       | 3.7        | 1.23       |
| Example 2 (A/dm <sup>2</sup> )       | 27.78      | 2.36        | 13.89      | 13.89       | 3.7        | 1.23       |
| Example 3 (A/dm <sup>2</sup> )       | 27.78      | 2.27        | 13.89      | 13.89       | 3.7        | 1.23       |
| Comparative                          | 27.78      | 1.23        | 13.89      | 9.26        | 4.94       | 1.23       |
| Example 1 (A/dm <sup>2</sup> )       |            |             |            |             |            |            |
| Comparative                          | 8.33       | 25.93       | 33.33      | 3.7         | 2.47       | 1.23       |
| Example 2 (A/dm <sup>2</sup> )       |            |             |            |             |            |            |

As shown in FIG. 4 and FIG. 5, the micro-rough surface of Example 1 has a plurality of micro-crystal clusters, each of which is composed of particles having a particle diameter less than 0.5  $\mu\text{m}$ , and the micro-crystal clusters have relatively larger spacing between each other. It is observed from the cross-sectional view that the micro-rough surface includes a plurality of V-shaped grooves spaced apart from each other and each having a depth less than 0.6  $\mu\text{m}$ . The micro-crystal clusters have a uniform distribution and most thereof are aggregated at the tops of the peaks (i.e., between the V-shaped grooves).

As shown in FIG. 6 and FIG. 7, the surface of the CF-T4X-SV copper foil is uniformly covered by a plurality of micro-crystals each having a particle diameter greater than 1  $\mu\text{m}$ ; and the micro-crystals do not aggregate with each other to form clusters. It is observed from the cross-sectional view that the micro-crystals are uniformly distributed on the surface and do not aggregate at certain locations. In addition, each of the micro-crystals has an average height greater than 1.5  $\mu\text{m}$ .

As shown in FIG. 8 and FIG. 9, the surface of the HS1-M2-VSP copper foil is uniformly covered by a plurality of micro-crystals each having a particle diameter greater than 0.5  $\mu\text{m}$ ; and most of the micro-crystals are spaced apart from each other and a few of the micro-crystals aggregate with each other to form clusters. It is observed from the cross-sectional view that the micro-crystals have relatively larger spacing between each other and are uniformly distributed on the surface and do not aggregate at certain locations. In addition, each of the micro-crystals has an average height between 1  $\mu\text{m}$  and 2  $\mu\text{m}$ .

15 observed that the micro-roughened electrolysis copper foil of the present disclosure has good bonding strength relative to the substrate and facilitates the performing of subsequent processes while maintaining the product yield.

20 With respect to the insertion loss performance, the insertion losses of the copper foil substrates of Examples 1 to 3 at 8 GHz to 30 GHz are substantially better than the insertion losses of the copper foil substrates of Comparative Examples 1 to 4. It is worth mentioning that, the present disclosure has better insertion loss performance than commercial products (e.g., Comparative Examples 3 and 4) at high-frequency ranges greater than 12.89 GHz. It is worth mentioning that, signal losses at high frequencies can be significantly reduced by controlling the surface profile of the 25 micro-rough surface and adjusting the Rlr value to less than 1.059. In addition, it can be found that as the Rlr value gets lower, the signal losses are correspondingly reduced.

30 It is evident from the above description that the micro-roughened electrolysis copper foil can further optimize the insertion loss performance to significantly reduce the signal losses while maintaining good peel strength.

35 The foregoing description of the exemplary embodiments of the disclosure has been presented only for the purposes of 40 illustration and description and is not intended to be exhaustive or to limit the disclosure to the precise forms disclosed. Many modifications and variations are possible in light of the above teaching.

The embodiments were chosen and described in order to explain the principles of the disclosure and their practical

TABLE 2

|                        | Examples  |        |        | Comparative Examples |        |        |        |        |
|------------------------|-----------|--------|--------|----------------------|--------|--------|--------|--------|
|                        | 1         | 2      | 3      | 1                    | 2      | 3      | 4      |        |
| Peel strength (lb/in)  | 3.96      | 4.04   | 4.12   | 2.98                 | 3.02   | 3.86   | 4.13   |        |
| Rlr                    | 1.04      | 1.051  | 1.059  | 1.16                 | 1.25   | 1.06   | 1.46   |        |
| Insertion loss (dB/in) | 4 GHz     | -0.198 | -0.199 | -0.199               | -0.223 | -0.241 | -0.200 | -0.190 |
|                        | 8 GHz     | -0.304 | -0.308 | -0.310               | -0.342 | -0.367 | -0.311 | -0.311 |
|                        | 12.89 GHz | -0.408 | -0.423 | -0.429               | -0.458 | -0.493 | -0.430 | -0.454 |
|                        | 16 GHz    | -0.499 | -0.516 | -0.530               | -0.560 | -0.605 | -0.530 | -0.561 |
|                        | 20 GHz    | -0.598 | -0.618 | -0.628               | -0.670 | -0.729 | -0.638 | -0.696 |
|                        | 25 GHz    | -0.730 | -0.752 | -0.770               | -0.817 | -0.897 | -0.783 | -0.881 |
|                        | 30 GHz    | -0.866 | -0.910 | -0.929               | -0.969 | -1.073 | -0.940 | -1.080 |

As shown in Table 2, with respect to the peel strength performance, the peel strengths of the copper foil substrates of Examples 1 to 3 are at least 3.96 lb/in that is between the peel strengths of the copper foil substrates of Comparative Examples 3 and 4 (i.e., commercial copper foils) and exceed the industry standard of 3 lb/in by at least 32%. It can be

65 application so as to enable others skilled in the art to utilize the disclosure and various embodiments and with various modifications as are suited to the particular use contemplated. Alternative embodiments will become apparent to those skilled in the art to which the present disclosure pertains without departing from its spirit and scope.

## 11

What is claimed is:

1. A micro-roughened electrodeposited copper foil comprising a micro-rough surface that has a plurality of peaks, a plurality of V-shaped grooves and a plurality of micro-crystal clusters, wherein each of the V-shaped grooves having an average depth less than 1  $\mu\text{m}$  is defined by adjacent two of the peaks, and the micro-crystal clusters are correspondingly located on the tops of the peaks and each thereof has an average height less than 1.5  $\mu\text{m}$ ;

wherein the micro-rough surface of the micro-roughened electrodeposited copper foil has an Rlr value less than 1.06, and the Rlr value satisfies the equation of  $\text{Rlr}=\text{Rlo}/\text{L}$ , where Rlo represents a measured profile length and L represents a measured distance.

2. The micro-roughened electrodeposited copper foil according to claim 1, wherein each of the micro-crystal clusters is composed of a plurality of micro-crystals grouped together, and has an average height of less than 1.3  $\mu\text{m}$ , and each of the micro-crystals has an average diameter less than 0.5  $\mu\text{m}$ .

3. The micro-roughened electrodeposited copper foil according to claim 2, wherein each of the micro-crystal clusters has an average number of the micro-crystals, being less than 15, that are stacked in a height direction of the micro-crystal clusters, and has an average maximum width less than 5  $\mu\text{m}$ , and a portion of the micro-crystal clusters are formed with a branch structure.

4. The micro-roughened electrodeposited copper foil according to claim 1, wherein the Rlr value of the micro-rough surface of the micro-roughened electrodeposited copper foil is less than 1.055.

5. The micro-roughened electrodeposited copper foil according to claim 2, wherein the Rlr value of the micro-rough surface of the micro-roughened electrodeposited copper foil is less than 1.055.

6. The micro-roughened electrodeposited copper foil according to claim 3, wherein the Rlr value of the micro-rough surface of the micro-roughened electrodeposited copper foil is less than 1.055.

7. A copper foil substrate, comprising:

a substrate; and  
a micro-roughened electrodeposited copper foil including a micro-rough surface attached to the substrate, the micro-rough surface having a plurality of peaks, a plurality of V-shaped grooves and a plurality of micro-crystal clusters, wherein each of the V-shaped grooves

## 12

has an average depth less than 1  $\mu\text{m}$  is defined by adjacent two of the peaks, and the micro-crystal clusters are correspondingly located on the tops of the peaks and each thereof has an average height less than 1.5  $\mu\text{m}$ ;

wherein the copper foil substrate has an insertion loss between 0 and -0.635 dB/in at 20 GHz;

wherein the micro-roughened electrodeposited copper foil has a peel strength greater than 3 lb/in relative to the substrate.

8. The copper foil substrate according to claim 7, wherein the copper foil substrate has an insertion loss between 0 and -0.935 dB/in at 30 GHz.

9. The copper foil substrate according to claim 8, wherein the copper foil substrate has an insertion loss between 0 and -0.31 dB/in at 8 GHz, an insertion loss between 0 and -0.43 dB/in at 12.89 GHz, and an insertion loss between 0 and -0.53 dB/in at 16 GHz, and the peel strength of the copper foil substrate relative to the substrate is greater than 3.5 lb/in.

10. The copper foil substrate according to claim 9, wherein the insertion loss of the copper foil substrate at 12.89 GHz is between 0 and -0.42 dB/in, the insertion loss of the copper foil substrate at 16 GHz is between 0 and -0.52 dB/in, the insertion loss of the copper foil substrate at 20 GHz is between 0 and -0.63 dB/in, the insertion loss of the copper foil substrate at 30 GHz is between 0 and -0.92 dB/in, and the peel strength of the copper foil substrate relative to the substrate is greater than 3.9 lb/in.

11. The copper foil substrate according to claim 7, wherein each of the micro-crystal clusters has an average maximum width less than 5  $\mu\text{m}$  and the average height thereof is less than 1  $\mu\text{m}$ , a portion of the micro-crystal clusters are formed with a branch structure, and each of the micro-crystal clusters is composed of a plurality of micro-crystals grouped together and each of the micro-crystals has an average diameter less than 0.5  $\mu\text{m}$ , and wherein the micro-rough surface of the micro-roughened electrodeposited copper foil has an Rlr value less than 1.06, and the Rlr value satisfies the equation of  $\text{Rlr}=\text{Rlo}/\text{L}$ , where Rlo represents a measured profile length and L represents a measured distance.

12. The copper foil substrate according to claim 7, wherein the substrate has a dielectric constant (Dk) less than 3.8 and a dissipation factor (Df) less than 0.002 at 1 GHz.

\* \* \* \* \*